

June 25, 1946.

P. F. MUMMA ET AL  
METHOD OF CASTING INGOTS  
Filed Nov. 16, 1943

2,402,833



INVENTORS.  
PAUL F. MUMMA  
ARTHUR W. THORNTON  
by: *John E. Jackson*  
ATTORNEY.

## UNITED STATES PATENT OFFICE

2,402,833

## METHOD OF CASTING INGOTS

Paul F. Mumma, McKeesport, and Arthur W. Thornton, Pittsburgh, Pa., assignors to National Tube Company, a corporation of New Jersey

Application November 16, 1943, Serial No. 510,532

7 Claims. (Cl. 22—216)

1

The present invention relates to an improved method of casting ingots, a primary object of the invention being to make possible the production of steel ingots in which the metallurgical pipe cavity is unoxidized and is free from slag or other contaminating non-metallic or metalloid materials.

A further object of the invention is to reduce the depth of the metallurgical pipe cavity insofar as this may be practical without resorting to the use of elaborate and expensive hot topping practices and without incurring the economic losses incident to the high ingot top discards required on conventional hot-topped ingots.

The above and related objectives of the invention will be more fully apparent from consideration of the following specification and claims when read in connection with the accompanying drawing, in which:

Figure 1 is a plan view of the apparatus for carrying out one of the essential steps of the improved method.

Figure 2 is a sectional view on line II—II of Figure 1, illustrating the manner of gently applying a coolant to the top crust formed on an ingot immediately after teeming.

Figure 3 is an elevation of the apparatus shown in Figure 1, viewed in the direction of the arrow 3 thereof.

Figure 4 is a section similar to Figure 2, illustrating a further essential step of applying an insulating material to the solidified top crust of the ingot.

In the conventional practice usually followed for the production of steel ingots of ordinary commercial grade (as distinguished from special quality steels receiving expensive and at times elaborate "hot topping treatment"), the ingot molds are filled with liquid steel to the desired height, and this molten metal solidifies into an ingot with no further special treatment, in accordance with the natural laws governing the solidification phenomenon. As is well known to those skilled in the art, when this conventional pouring practice is used on semi-killed or killed steels, the resulting ingot contains a deep, roughly cone-shaped cavity, generally referred to as a metallurgical pipe, in its top portion. This pipe results from a volumetric contraction obtained in the transition of the metal from the molten to the solid state. The top of the pipe is covered over by a crust of initially solidified metal which, under optimum conditions, should be continuous and free from openings leading to the metallurgical pipe. In actual practice, however, many

2

ingots fail to achieve this ideal condition upon freezing, but on the contrary the crusts are somewhat porous, having objectionable so-called "rat holes," permitting access to the interior of the metallurgical pipe. During the subsequent heating of ingots with porous crusts in the soaking pit furnaces, the pipe becomes oxidized on its inner surface and is contaminated with slag and molten oxides that flow down these passageways into the pipe. When the teachings of our invention, hereinafter more fully set forth, are followed, the top crust of the ingot spanning the metallurgical pipe is uniformly non-porous, and thus an important advantage arises by the exclusion from the pipe of oxidized portions and the exclusion from the pipe of slag or oxides such as inherently collect within the pipe according to conventional practice.

It is well known to those skilled in the art of making, shaping, and treating steel products, that the piped ends of ingots are cropped off, thus producing a large amount of heavy scrap. However, in the rolling of certain steel products such as seamless steel tubing produced by the rotary piercing process, it is found that within reasonable limits a clean, unoxidized and slag-free pipe portion of an ingot is not detrimental to the quality of the finished product, and hence if this condition can be maintained, which is made possible under the herein claimed invention, a higher ingot-to-finished product yield is achieved.

Referring to the drawing, in carrying out our novel method, molten steel contained in an overhead conventional portable ladle 10 is teemed into 35 a conventional ingot mold 12. Immediately after the teeming, we gently apply a coolant so as to insure that a non-porous top crust 14 is formed on the ingot 16. The coolant generally employed is water, and we deem it important to initially 40 apply the water so as to gently flow it over the top of the molten metal quickly after teeming. As suggested in Figures 1 and 2, a coolant such as water may be applied by discharging a plurality of jets 20 from a pipe 22 obliquely downward, so that the jets first impinge on the inner face 24 of the mold opposite the pipe 22. This water then gradually and gently floats over the top of the molten steel forming the crust 14.

The volume of water supplied is under control 50 of a valve 28 located in pipe 26 leading to a suitable source of water or other coolant. The water or other coolant is effective to seal the initial top crust 14 of the ingot, thus preventing the formation of passageways or rat holes leading into the metallurgical pipe 18. The quantity of water

used varies somewhat with the ingot size. For example, we have found that approximately 10 gallons should be used on a 10,000-pound ingot having a top area of 575 square inches. It is deemed essential that the water or other coolant be applied quickly after completion of the teeming, preferably within about two minutes. It is also considered important that the water application be made in a gentle manner so as not to rupture the initial, extremely tender solidified film which eventually becomes the thicker crust 14. We have found that this gentle initial water application can be effectively made by the relatively simple and inexpensive apparatus such as shown in Figures 1, 2, and 3 of the drawing, 15 which is nothing more than a drilled pipe with a control valve therein, the nozzles or orifices in the pipe being disposed at the proper angle to impinge the water jet first on the side wall of the mold, as indicated in Figure 2, so that thereafter the water body is slowly and gently flowed over the molten steel. Following the initial gentle application, for example, after the first 10 per cent of the total water used is applied, the remainder of the total water may be added in 20 any manner found most convenient. Other means of spraying could, of course, be used during the initial application, and if desired the entire quantity of water could be placed on the ingot top by discharging the water through a 25 perforated pipe such as shown at 22. The net result of the gentle application of water or other coolant to the top of the molten metal which eventually forms the ingot, it will be appreciated, is to form an impervious crust 14 spanning the 30 pipe or cavity 18 so as to prevent or minimize oxidation of the surface of the pipe and to exclude oxidized slag or other contaminating non-metallic materials such as normally collect within the pipe under prior practices where no special provision is made for their exclusion.

After the impervious crust 14 is formed by the gentle application of the coolant, an insulating material such as indicated at 32 in Figure 4 is applied to the top crust 14. This insulating material is effective to restrict heat dissipation from the exposed ingot top surface, and thus assist in maintaining a portion of the ingot top volume (beneath the solidified crust 14) in a molten state for a longer-than-normal period of time, so that this molten metal, by gravitating toward the body of the ingot, will partially compensate for the volumetric shrinkage taking place in the ingot and hence reduce the depth of the metallurgical pipe. The insulating material 32 may be one or more of a variety of inert or combustible materials such as sand, pulverized brick, dehydrated lime, limestone or dolomite dust, coke dust, fine coal, straw, grain hulls, cork, etc., its principal requirement being that either by blanketing effect or by exothermic action, or both, it acts to restrict heat flow from the top surface of the ingot. No question of ingot metal contamination is involved since the prior water-sealing operation prevents access of the insulating material, or its reaction products, to the molten metal beneath the water-sealed ingot top crust.

Heretofore, when using conventional hot-topping practices, the cropped-off or discarded tops of the ingots are normally of the order of 70 from 12 to 20 per cent of the weight of the ingot. An important advantage of the herein claimed invention is that a much smaller portion of the ingot need be discarded, this being due to the fact that there is no mechanical discontinuity

in the outside ingot surface, such as occurs at the juncture of ingot body and hot top section of a conventionally hot-topped ingot, and, as a result of the special method step followed, the pipe is devoid of objectionable oxide or metalloid inclusions.

While we have described quite precisely certain specific steps which a reduction to practice has shown to be highly advantageous, and have illustrated apparatus found to be practical and well suited for carrying out the herein claimed method, it is to be understood that the detailed disclosure and drawing are to be interpreted in an illustrative rather than a limiting sense, since various modifications may be resorted to by those skilled in the art without departing from the spirit and scope of the invention as defined in the appended claims.

We claim:

1. In the casting of ingots, the method which comprises teeming molten metal into an ingot mold, applying a coolant to the top surface of the ingot immediately after said teeming step so as to effectively seal the initial top crust of the ingot, and covering the solidified top crust with an insulating material to restrict heat dissipation from the exposed ingot top surface and thus assist in maintaining a portion of the ingot top beneath the solidified crust in a molten state for a longer-than-normal period of time, so that this molten metal, by gravitating toward the body of the ingot, will partially compensate for the volumetric shrinkage taking place there and hence reduce the depth of the metallurgical pipe.

2. In the casting of ingots, the method which comprises teeming molten metal into an ingot mold, gently applying a coolant to the top surface of the ingot immediately after said teeming step so as to effectively seal the initial top crust of the ingot, and covering the solidified top crust with an insulating material to restrict heat dissipation from the exposed ingot top surface to thus assist in maintaining a portion of the ingot top volume in a molten state for a sufficient period of time to allow the molten metal to gravitate toward the body of the ingot so as to partially compensate for volumetric shrinkage taking place there and hence reduce the depth of the metallurgical pipe.

3. In the casting of ingots, the method which comprises teeming molten metal into an ingot mold, directing a jet of water against a wall of the mold cavity so as to gently apply the water to the top surface of the ingot immediately after said teeming step so as to form an impervious initial top crust on the ingot, and covering the top crust with an insulating material to restrict heat dissipation from the exposed ingot top surface and thus assist in maintaining a portion of the ingot top volume beneath the solidified crust in a molten state for a longer-than-normal period of time, so that this molten metal, by gravitating toward the body of the ingot, will partially compensate for the volumetric shrinkage taking place there and hence reduce the depth of the metallurgical pipe.

4. In the casting of ingots, the method which comprises teeming molten metal from an overhead source into an ingot mold, impinging a coolant against an inner wall of the ingot mold so as to gently apply said coolant to the top surface of the teemed metal immediately after said teeming step so as to form an impervious top crust on the ingot, and covering the thus-formed top crust with comminuted insulating material

to retard the dissipation of heat from the top surface of the ingot.

5. In the casting of ingots, the method which comprises teeming molten metal from an overhead source into an ingot mold, directing water at a low angle against the inner wall of the ingot mold, so as to gently apply said water to the top surface of the ingot immediately after said teeming step so as to form an initial impervious top crust on the ingot, and covering the

10

said top crust with an insulating material to retard the dissipation of heat from the top surface of the ingot.

6. In the casting of ingots, the method which comprises teeming molten metal from an overhead source into an ingot mold, gently applying a determined amount of coolant thereto so as to quickly form an impervious top crust thereon to obtain a pipe free of oxidation and slag and covering the said top crust with an insulating material to retard the dissipation of heat therefrom, thereby reducing the extent of the pipe so that a large percentage of the ingot can be rolled into seamless tubing and the like.

PAUL F. MUMMA.  
ARTHUR W. THORNTON.